

Sept. 16, 1930.

A. E. VILLAREJO

1,776,015

PRINTING PLATE AND PROCESS OF PRODUCING THE SAME

Filed Oct. 21, 1929



Inventor  
By Alfred E. Villarejo  
Bottom, Hadley, Ladd, Weston and Nichols  
ATTORNEYS

## UNITED STATES PATENT OFFICE

ALFRED E. VILLAREJO, OF MILWAUKEE, WISCONSIN, ASSIGNOR OF ONE-HALF TO  
RUDOLF P. ZETTINIG, OF MILWAUKEE, WISCONSIN

## PRINTING PLATE AND PROCESS OF PRODUCING THE SAME

Application filed October 21, 1929. Serial No. 401,032.

This invention relates in general to the production of printing plates by electrodeposition and more particularly to the direct production of such plates on a metallic original.

In applying graining, simulating wood graining, or other ornamentation to the metal panels of automobile bodies, it is the usual practice to have a positive metal plate or original on which the graining or design has been produced. In the case of wood graining, the original metal plate has ridges and valleys, conforming to the contour of the graining. The plate is inked and after any excess of the ink is removed, a roller is run over the plate and then run over the metal panel of the automobile body so that the design is transferred to the metal panel of the automobile body.

20 The production of the positive metal plates from which the impressions are transferred by the roller is a source of difficulty and expense, especially where these plates are of any substantial size, as they frequently must 25 be in connection with the graining of, or the application of other ornamentation to, certain automobile panels.

In this art the practice heretofore has been to produce a design on the original metal 30 plate by a photographic (half-tone) process, and then transfer the impression or design from the original to a body of wax by pressing the body of wax against the original. The surface of the wax which has the impression produced thereon in this way is then 35 coated with graphite and then placed in an electro-plating bath and subjected to the electro-plating process so that a coating of copper is then deposited over the graphite 40 surface of the wax. The wax is then melted out of the deposited plate and this plate is the one that is inked and from which the impression is transferred to the automobile panel by the transferring roller.

45 One of the principal objects of the present invention is to dispense with the use of the wax and to deposit the metal in the electro-plating bath, directly onto the original metal plate produced by the usual photographic process. The great difficulty that has here-

tofore stood in the way of the direct production of printing plates in this manner has resided in the fact that where the metal is directly deposited on the original in the electro-plating bath, it is impossible to strip off the 55 deposited plate. In some arts it has been proposed to use separating or stripping films of silver compounds, lead, cobalt, hydrocarbons or the like, but all of these films are unsatisfactory for various reasons such as 60 expense, loss of detail, damage to the original or the like.

The present invention produces a separating or stripping film on the original in a speedy and comparatively inexpensive manner and does this without damage to the original and without loss of detail and yet insures the easy stripping off of the electro-lytically deposited plate.

Other objects and advantages reside in certain novel features which will be hereinafter more fully described, and particularly pointed out in the appended claims, reference being had to the accompanying drawing forming a part of this specification and in 75 which:

Figure 1 is a plan view of an original from which printing plates are to be produced;

Figure 2 is a view in section of line 2-2 80 of Figure 1;

Figure 3 is a figure similar to Figure 2, but illustrating the coating formed on the surface of the original plate which carries the design, the coating being exaggerated for 85 the sake of clearness;

Figure 4 is a diagrammatic view illustrating how the negative plate is deposited on the original;

Figure 5 is a view similar to Figure 3, 90 showing how the positive printing plate is deposited on the negative plate; and

Figure 6 is a diagrammatic view in perspective illustrating how the inked roller is used with the positive printing plate produced in accordance with the present invention.

Referring then to the drawings, it will be seen that an original metal plate 1, preferably of copper, is provided and has a design 100

etched or otherwise formed on the surface 2 thereof by means of a conventional photographic process. The surface 2, on which the design is formed or carried, is first subjected to a bath of ammonium polysulphide  $(\text{NH}_3)_2\text{S}_2$ , either by immersing the surface 2 in a concentrated solution of ammonium polysulphide or by subjecting it to a light washing therewith, the latter being preferred. The ammonium polysulphide reacts with the copper of the surface 2 of the plate 1 to produce a very light film or coating of copper sulphide on the surface of the original copper plate carrying the design. After the treatment with the ammonium polysulphide, the plate is dried—atmospheric drying being sufficient—and is then washed gently with distilled water. Following this, the plate is baked to harden the thin film of copper sulphide produced thereon by the ammonium polysulphide.

The plate, thus prepared, is placed in an ordinary electro-plating bath as illustrated diagrammatically in Figure 4 and a shell of copper 3 is deposited thereon in the ordinary way. When sufficient metal has been deposited to make the shell 3 of the desired thickness, the plate and shell are removed from the bath and the shell 3 is stripped from the original plate 1. The shell will come off easily due to the use of the sulphide coating on the original plate. The shell 3 is, however, a negative. In order to produce a positive from the shell 3 the process is repeated and is identical with the process above described, except that the thin shell 3 must be placed on an appropriate backing shown at 5 in Figure 5 unless it is made sufficiently heavy to dispense with the backing. The shell 3 is, however, treated with ammonium polysulphide to produce the thin coating or film of copper sulphide thereon and is then dried, washed, baked and put in an electro-plating bath as illustrated in Figure 5 so that the positive printing plate, or shell 4, is deposited on the shell 3. This shell 4 can also be easily stripped from the shell 3, and may be later used as indicated in Figure 6, to apply the impression to the transferring roller 6 which in turn applies the impression to the panel to be ornamented.

As indicated, ammonium polysulphide is preferably the reagent used to produce the copper sulphide coating as it produces a hard film that will not flake off and that will not impair the design. However, other reagents such as potassium sulphide or sodium sulphide may be employed to produce the coating.

It is to be noted that the copper sulphide coating is formed on and of the metal which constitutes the features of the original design and is an integral part of such features. In other words, the copper sulphide coating is a result of the transformation of the sur-

face metal of the copper plate and consequently there is no loss in detail in the design on such surface. It is coherent and will not rub off or be displaced and as it is a constituent part of the features of the design and is of uniform thickness it does not deprive the design of any of its detail, nor does it impair the same in any way. Further, the film is a good conductor of electricity so as not to interfere with the electro-plating process. The invention dispenses with the use of the expensive and temporary wax or gutta percha, avoids the annoyance and difficulties experienced from using graphite dust with such wax or gutta percha and provides means whereby a great many, at least thirty, printing plates can be made from one negative.

Finally, the coating is produced at a comparatively slight expense and without loss of time or the expenditure of any material amount of labor or the exercise of any special skill.

The invention claimed is:

1. The herein described process of producing printing plates from an original copper plate which consists in first, subjecting the surface of the original copper plate carrying the design to a bath of ammonium polysulphide to form a thin film of copper sulphide on and as a part of the metal of the plate that constitutes the features of the design, drying and washing the original plate, baking the original plate to harden the film thereon, then electrodepositing a negative copper plate on the film coated original, stripping of the negative plate from the original, similarly coating the surface of the negative plate with copper sulphide, and finally electro-depositing a positive printing plate on the film coated surface of the negative plate.

2. The herein described process of producing printing plates from an original copper plate which consists in first, subjecting the surface of the original copper plate carrying the design to a bath of ammonium polysulphide to form a thin film of copper sulphide thereon and as a part of the metal of the plate that constitutes the features of the design, drying and washing the original plate, and baking the original plate to harden the design thereon.

In witness whereof, I hereto affix my signature.

ALFRED E. VILLAREJO. 120